

July 25, 1972

F. KALWAITES  
NONWOVEN FABRIC COMPRISING DISCONTINUOUS GROUPS  
OF SMALL HOLES CONNECTED BY RIBBONS  
DEFINING LARGE HOLES

3,679,535

Filed March 24, 1970

4 Sheets-Sheet 1

Fig. 1.

Machine direction →



Fig. 2.



INVENTOR  
FRANK KALWAITES  
BY *John J. Neenan*  
ATTORNEY

July 25, 1972

F. KALWAITES

3,679,535

NONWOVEN FABRIC COMPRISING DISCONTINUOUS GROUPS  
OF SMALL HOLES CONNECTED BY RIBBONS  
DEFINING LARGE HOLES

Filed March 24, 1970

4 Sheets-Sheet 2



INVENTOR  
FRANK KALWAITES

BY

ATTORNEY

July 25, 1972

F. KALWAITES

3,679,535

NONWOVEN FABRIC COMPRISING DISCONTINUOUS GROUPS  
OF SMALL HOLES CONNECTED BY RIBBONS  
DEFINING LARGE HOLES

Filed March 24, 1970

4 Sheets-Sheet 3

T19.5.



T19.9.



T19.11.



T19.10.



INVENTOR  
FRANK KALWAITES  
BY *Frank Kalwaites*  
ATTORNEY

July 25, 1972

F. KALWAITES

**3,679,535**

**F. KALWATTES**  
NONWOVEN FABRIC COMPRISING DISCONTINUOUS GROUPS  
OF SMALL HOLES CONNECTED BY RIBBONS  
DEFINING LARGE HOLES

Filed March 24, 1970

4 Sheets-Sheet 4



**INVENTOR**  
**FRANK KALWAITES**

BY

**ATTORNEY**

## 1

3,679,535

**NONWOVEN FABRIC COMPRISING DISCONTINUOUS GROUPS OF SMALL HOLES CONNECTED BY RIBBONS DEFINING LARGE HOLES**

Frank Kalwaites, Somerville, N.J., assignor to

Johnson & Johnson

Filed Mar. 24, 1970, Ser. No. 22,290

Int. Cl. D04h 1/46, 1/70

U.S. CL. 161—109

7 Claims

### ABSTRACT OF THE DISCLOSURE

A nonwoven fabric having a plurality of patterns of groups of fiber segments that alternate and extend throughout the fabric. The first pattern is of yarn-like bundles of fiber segments which define holes or apertures or other areas of low fiber density located in first discontinuous portions of the fabric. These discontinuous portions of the fabric are interconnected by ribbon-like groups of aligned fiber segments that form a second pattern in second discontinuous portions of the fabric.

The present invention relates to nonwoven fabrics and more particularly to patterned nonwoven fabrics made from a layer of fibrous material such as a fibrous web wherein the individual fiber elements are capable of moving under the influence of applied fluid forces. The fabric contains a plurality of patterns of different types of groups of fiber segments that alternate and extend throughout the fabric.

### BACKGROUND OF THE INVENTION

For a number of years, there have been known various type of foraminous or apertured nonwoven fabrics made by processes involving the rearrangement of fibers in a starting web or layer of nonwoven fibers. Some of these fabrics and methods of manufacture are illustrated, shown, and described in U.S. Pats. 2,862,251; 3,081,500; 3,081,512; 3,081,514; 3,081,515; 3,025,585; and 3,033,721. The fabrics disclosed and claimed in the patents just listed contain apertures or holes or other areas of low fiber density which are often outlined by interconnected bundles of fibrous elements wherein the fiber segments within the bundle are closely associated and substantially parallel and have a yarn-like configuration. The term "areas of low fiber density" is used in this specification and claims to include both areas in which relatively few fibers in comparison to the rest of the fabric are found, and apertures (holes) that are substantially or entirely free of fibers. Such fabrics are sometimes referred to as "bundled rearranged" nonwoven fabrics.

Bundled rearranged nonwoven fabrics have been made commercially for many years. In most instances, these fabrics have had an overall pattern of holes or other low fiber density areas throughout the fabric.

A method for producing bundled rearranged nonwoven fabric is to support a loose fibrous web or layer on a permeable backing member and apply sets of opposing fluid forces to the layer while thus supported. The fluid by which such forces are applied passes through the fibrous layer, over the backing member, and then through the backing member to pack various groups of the fiber elements and place these elements into closer proximity and substantial parallelism to form interconnected bundles of fiber segments. In accomplishing this result, the fluid forces usually are applied over the entire surface of the loose fibrous web or layer and uniformly over and through the permeable backing or support member to produce fiber bundles uniformly over the entire fabric. In some instances, patterns can be made in the fabric by not applying

## 2

ing fluid forces in predetermined areas of the fibrous layer, thereby preventing rearrangement in these areas.

### SUMMARY OF THE INVENTION

5 I have discovered a novel nonwoven fabric which comprises a layer of intermingled fibers with the fibers arranged to form a plurality of patterns that alternate and extend throughout the fabric. The first pattern is of yarn-like bundles of fiber segments which define apertures or holes or other areas of low fiber density in first discontinuous portions of the fabric. Each of the areas of low fiber density in the first pattern are defined by a plurality of yarn-like bundles of fiber segments. The fiber segments in each of these bundles are closely associated with other fiber segments in the bundle and lie generally parallel to the longitudinal axis of the bundle. The yarn-like bundles of fiber segments are interconnected to other such bundles at junctures by groups of fibers common to a plurality of bundles. The fibers at these junctures are oriented in a plurality of diverse directions.

10 The first discontinuous portions of the fabric are interconnected by ribbon-like groups of substantially aligned fiber segments. The interconnecting groups are located in second discontinuous portions of the fabric. The interconnecting groups form a second pattern of aligned fiber segments which will alternate with the first pattern of groups of fiber segments and extend throughout the fabric.

15 In some embodiments of the present invention, the interconnecting groups of substantially aligned fiber segments in the second discontinuous portions of the fabric define another plurality of holes or apertures or other areas of low fiber density that are located in third discontinuous portions of the fabric.

20 Surprisingly, even though my new fabric has a plurality of patterns that alternate and extend throughout the fabric, the patterns have substantial regularity which aids in giving the fabric considerable aesthetic appeal. Not only does my new fabric have substantial uniformity in its arrangement of holes or apertures or other areas of low fiber density, but unexpectedly, my new fabric has uniformity in the pattern of bundles of fiber segments which define the areas of low fiber density in the first discontinuous portions of the fabric and in the pattern of ribbon-like groups of substantially aligned fiber segments which interconnect the discontinuous portions of the fabric that form the first pattern.

### METHOD OF MAKING THE FABRIC OF THIS INVENTION

25 In the method of making the fabric of this invention, the layer of fibrous starting material is supported in a fiber rearranging zone in which fiber movement in directions parallel to the plane of said fibrous material is permitted in response to applied fluid forces. Streams of rearranging fluid, preferably water, are projected into the fibrous layer at entry zones spaced from each other adjacent one surface of the layer, each of the entry zones having a width at its narrowest part equal to at least about ten times, and preferably about twenty or more times, the average diameter of the fibers of the fibrous starting material. These streams of rearranging fluid are passed through the layer of fibrous starting material as it lies in the rearranging zone, to effect movement of at least some segments of the fibers transverse to the direction of travel of the projected streams.

30 In the next step of the method, the passage of first portions of the rearranging fluid out of the fibrous layer is blocked at continuous barrier zones located adjacent the opposite surface of the fibrous layer, and, at the same time, those portions of fluid are deflected sidewise towards the other portions of the rearranging fluid and are actively mingled with the latter. Each of the barrier zones

has a width at its narrowest part equal to at least about the width of one of the entry zones at its narrowest part. All the portions of intermingled rearranging fluid are then passed out of the rearranging zone through spaced, discontinuous, foraminous zones defined by the continuous barrier zones and each having an area at least about three times, and preferably about four or more times, the area of one of the entry zones.

The passage of the rearranging fluid through the layer of fibrous starting material as just described moves some of the fiber segments that are in registry with the continuous barrier zones into the foraminous zones, and positions those fiber segments with other fiber segments in a pattern of yarn-like bundles which define areas of low fiber density in the foraminous zone. In addition, the rearranging fluid moves other fiber segments that are in registry with the barrier zones into substantial alignment in flat, ribbon-like groups of fiber segments in bridging positions extending between the discontinuous foraminous zones.

In one method of manufacturing my new nonwoven fabric, a starting layer of fibrous material, the individual fibrous elements of which are capable of movement under the influence of applied fluid forces, is subjected to fluid rearranging forces, preferably liquid, while the layer is supported on a permeable backing member. The backing member has a predetermined topography and has foraminous areas arranged in a discontinuous pattern that are interconnected by continuous imperforate areas. The fluid flows over and through the foraminous areas and only over the imperforate areas. This fluid flow causes counteracting components of force to act to rearrange fibers into groups of yarn-like fiber bundles above the foraminous areas of the backing means. This fluid flow also causes components of force to act on the fibrous layer to align fiber portions into groups in accordance with the pattern of imperforate areas of the backing member. These fiber portions generally align themselves in flat ribbon-like groups in such a manner as to span each imperforate area and connect immediately adjacent portions of the fabric lying above the foraminous areas of the backing member.

The basic method and apparatus for making the fibers of this invention are shown and described fully in my U.S. Pat. No. 2,862,251, issued Dec. 2, 1958. Full particulars of the basic invention as disclosed in that patent are incorporated in this application by reference, although some of those particulars are repeated here. In addition, the specific feature peculiar to the method and apparatus for making the fibers of the present invention—which is the use of a backing member—is described in detail in this application.

#### Starting material

The starting material used with the method or apparatus for making the fabrics of this invention may be any of the standard fibrous webs such as oriented card webs, isoweb, air-laid webs, or webs formed by liquid deposition. The webs may be formed in a single layer, or by laminating a plurality of the webs together. The fibers in the web may be arranged in a random manner or may be more or less oriented as in a card web. The individual fibers may be relatively straight or slightly bent. The fibers intersect at various angles to one another such that, generally speaking, the adjacent fibers come into contact only at the points where they cross. The fibers are capable of movement under forces applied by fluids such as water, air, etc.

To produce a fabric having the characteristic hand and drape of a textile fabric, the layer of starting material used may comprise natural fibers such as cotton, flax, etc.; mineral fibers such as glass; artificial fibers such as viscose rayon, cellulose acetate, etc.; or synthetic fibers such as the polyamides, the polyesters, the acrylics, the polyolefins, etc., alone or in combination with one another. The fibers used are those commonly considered textile

fibers; that is generally having a length from about  $\frac{1}{4}$  inch to about 2 to  $2\frac{1}{2}$  inches. Satisfactory products may be produced in accordance with this invention from starting webs weighing between 80 grains per square yard to 2000 grains per square yard or higher.

#### Apertured forming means

In one form of the method and apparatus for making the fabric of this invention, the fluid entry zones into the fiber rearranging zone are defined by an apertured forming means.

The apertured forming means used is solid throughout its area except for the forming apertures disposed longitudinally and transversely across the member. The forming apertures may have any desired shape, i.e., round, square, diamond, oblong, free form, etc.

The width at the narrowest part of each of the apertures of the apertured forming means must be large enough that streams of rearranging fluid passing through those apertures will be effective to separate groups of fiber segments into yarn-like bundles spaced sufficiently far apart to permit reliable visual resolution. Without such resolution, any bundle of fiber segments produced would seem to the person viewing the fabric to fuse or merge together with other such bundles, with the result that no clear pattern would be apparent in the fabric. To achieve such resolution, the width of each aperture at its narrowest part should be equal to at least about ten times, and preferably at least about twenty times, the average diameter of the fibers in the fibrous starting material.

The land areas of the apertured forming means that lie between and interconnect the forming apertures may be either narrow or broad in comparison to the forming apertures, as desired. Generally speaking, the narrower the land areas are, the more tightly compacted will be the yarn-like bundles of closely associated and substantially parallel fiber segments that are formed beneath those land areas.

#### Backing means having discontinuous foraminous portions

As already indicated, in one form of this invention the fibrous starting layer is supported on backing means having foraminous portions arranged in a discontinuous pattern, and continuous imperforate portions that lie between and interconnect the discontinuous foraminous portions to provide barrier zones against the passage of rearranging fluid out of the fiber rearranging zone. The width of each imperforate portion of the backing means at its narrowest part is equal to at least about the width of the narrowest part of an aperture of the apertured forming means with which the backing means is used. The foramina of the foraminous portions of the backing means are substantially smaller than the apertures of the apertured forming means.

The bridging of the imperforate portions of the backing means by aligned fiber segments referred to above is brought about by three factors—good drainage of the rearranging fluid from the fiber rearranging zone with no uncontrolled washing away of fibers, the accumulation and retention of groups of fiber segments at spaced points across the backing means, and the pulling taut of other fiber segments that extend between such groups and are anchored by them at a plurality of points along their lengths.

Good drainage is achieved by avoiding the use of too much rearranging fluid and by employing discontinuous foraminous portions in the backing means that are large enough and not too widely spaced. As indicated above, the area of each of the discontinuous foraminous portions of the backing means should be at least about three times, and preferably four times, the area of an aperture of the apertured forming means. These foraminous portions should be closely enough spaced to each other that they occupy together at least about 20 percent, and preferably

about 30 percent or even more, of the total area of the backing means.

Accumulation and retention of fiber segments at spaced points across the backing means takes place when each foraminous portion of the backing means is large enough that a group of fibers can be accumulated and retained in the form of a plurality of yarn-like bundles of fiber segments which define areas of low fiber density.

The pulling taut of fiber segments between adjacent groups in which they are anchored is achieved by limiting the maximum spacing of the foraminous portions of the backing means. To establish two reliable anchor points for each individual fiber segment, the foraminous portions of the backing means should be spaced from other such portions immediately adjacent thereto by no more than about  $\frac{1}{3}$  the average length of the fibers being rearranged, and preferably no more than about  $\frac{1}{5}$  or  $\frac{1}{6}$  the length of the fibers. In general, this means that with  $1\frac{1}{2}$ " staple length fibers, each pair of foraminous portions of the backing means should be spaced, at their closest points, no more than about  $\frac{1}{2}$ " apart, and preferably no more than about  $\frac{1}{4}$ ".

In plan view, the discontinuous foraminous portions of the backing means may have any shape desired, i.e., circular, oval, diamond, square, etc.

The discontinuous foraminous portions may be flush with the imperforate portions of the backing means, or at a different elevation. If a three-dimensional effect is desired for the fiber grouping accumulated at each foraminous portion of the backing means, the continuous imperforate portions of the backing means may lie above the foraminous portions by as much as about  $\frac{1}{32}$ " or slightly higher. This difference in height must not be too great or it will interfere with the production of a pattern of yarn-like bundles of fiber segments above each discontinuous foraminous portion of the backing means.

In certain methods for producing the fabric of the present invention, each discontinuous foraminous portions of the backing means may be provided with a plurality of protuberances and troughs alternating across its surface in both the longitudinal and transverse directions. The tops of the protuberances should rise above the bottoms of the immediately adjacent troughs by a vertical distance equal to at least about three times the average diameter of the fibers in the layer of fibrous starting material. Preferably, the distance referred to should be equal to about ten times the average diameter of those fibers. When such a backing means is used, the apertured forming means may be eliminated, and the protuberances and troughs will produce a pattern of areas of low fiber density with each area defined by a plurality of yarn-like bundles. If such a backing means is used in conjunction with the apertured forming means, yet another pattern of yarn-like bundles is formed in the areas of low fiber density produced by the apertured forming means.

#### Rearranging fluid

The rearranging fluid for use in making fabrics of this invention is preferably water or a similar liquid, but it may be other fluids such as a gas, as described in my Pat. No. 2,862,251.

If desired, a vacuum may be applied at the exit side of the fiber rearranging zone to assist in moving the rearranging fluid through the fibrous starting material and in rearranging the fibers of the material into a patterned nonwoven fabric. This feature is most useful when the rearranging fluid is a liquid.

Even though some of the rearranging forces applied to the loose fibrous web in making my fabric are considerably different in magnitude than other forces applied to the loose fibrous web, these rearranging forces of disparate magnitude do not conflict or compete with each other but cooperate with and complement each other to produce uniformity and regularity in the areas of low

fiber density, the yarn-like fiber bundles, and the interconnecting flat, ribbon-like groups of aligned fiber segments. My new nonwoven fabrics can be made with patterns which simulate fancy woven and knitted fabrics and which even simulate lace, crocheted fabrics and the like.

#### BRIEF DESCRIPTION OF THE DRAWINGS

The invention will be more fully described in conjunction with the accompanying drawings wherein:

FIG. 1 is a photomicrograph of a fabric of the present invention at an original enlargement of 5 times.

FIG. 2 is a photomicrograph of another fabric of the present invention at an original enlargement of 5 times.

FIG. 3 is a schematic drawing of a fabric in accordance with the present invention.

FIG. 4 is a schematic drawing of another embodiment of the fabric in accordance with the present invention.

FIG. 5 is still another diagrammatic showing of a fabric in accordance with the present invention.

FIG. 6 is a diagrammatic showing in elevation of one type of apparatus for carrying out a method for producing the fabrics of the present invention.

FIG. 7 is an enlarged diagrammatic view of a portion of the backing means used in the apparatus of FIG. 6.

FIG. 8 is a cross-sectional view taken along line 8—8 of FIG. 7.

FIG. 9 is an enlarged fragmentary diagrammatic plan view of the foraminous portion of another backing means that can be used with the apparatus of FIG. 6, an aperture of the apertured forming means being shown in dashed lines.

FIG. 10 is a cross-sectional view taken along the line 10—10 of FIG. 5.

FIG. 11 is a cross-sectional view taken along line 11—11 of FIGS. 9 and 10.

#### DETAILED DESCRIPTION OF SPECIFIC EMBODIMENTS OF THE INVENTION

Referring to the photomicrograph in FIG. 1, there is shown a nonwoven fabric of the present invention. The fabric 20 includes a plurality of areas of low fiber density 21 in first discontinuous portions 22 of the fabric. The areas of low fiber density are defined by a first regular or predetermined pattern of yarn-like bundles 23 of fiber segments. The yarn-like bundles are interconnected to other such bundles at junctures 24 by fibers common to a plurality of the bundles. The first discontinuous portions of the fabric are interconnected by a second pattern of flat, ribbon-like 25 groups of substantially aligned fiber segments located in second discontinuous portions of the fabric. These interconnecting groups define a plurality of areas of low fiber density 26 in the fabric in third discontinuous portions of the fabric.

Referring to photomicrograph FIG. 2, a very similar fabric to that in FIG. 1 is shown. The fabric 30 has a plurality of areas of low fiber density 31 in first discontinuous portions 32 of the fabric. The areas of low fiber density are defined by a first regular or predetermined pattern of yarn-like bundles 33 of fiber segments, with the bundles being interconnected with other bundles at junctures 34 by fibers common to a plurality of the bundles. The first discontinuous portions of the fabric are interconnected by a second pattern of flat, ribbon-like groups 35 of substantially aligned fiber segments in second discontinuous portions of the fabric. These interconnecting groups form a plurality of areas of low fiber density 36 in third discontinuous portions of the fabric.

The major difference between the fabric shown in FIGS. 1 and 2 is that the fabric in FIG. 1 is made from an oriented card web, that is with the fibers generally aligned in the direction of the arrow shown, whereas fabric shown in FIG. 2 is made from an isoweb, that is, with the fibers randomly oriented. Because of this difference in original orientation, the areas of low fiber

density 26 in FIG. 1 are in some instances partially covered by a few fiber segments while the areas of low fiber density 36 in FIG. 2 are substantially free of fiber segments.

In FIG. 3 of the drawings, there is shown a schematic view of the fabric of FIG. 1. The fabric 40 includes a plurality of areas of low fiber density 41 in first discontinuous portions 42 of the fabric. Each of the areas of low fiber density is defined by a first regular or predetermined pattern of yarn-like bundles 43 of fiber segments. The yarn-like bundles 43 of fiber segments are interconnected with other bundles at junctures 44. These discontinuous portions of the fabric are arranged in a staggered pattern over the fabric.

The first discontinuous portions of the fabric are interconnected by a second regular or predetermined pattern of flat, ribbon-like groups 45 of substantially aligned fiber segments in second discontinuous portions of the fabric. These groups of fiber segments define areas of low fiber density 46 in third discontinuous portions of the fabric. The groups of fiber segments are disposed substantially uniformly about the periphery of each discontinuous portion at about the 5 and 11 o'clock positions and the 1 and 7 o'clock positions.

In FIG. 4, there is shown another embodiment of a nonwoven fabric according to the present invention. In this embodiment, the fabric 50 includes a plurality of areas of low fiber density 51 with the areas of low fiber density defined by a first pattern of yarn-like bundles 52 of fiber segments interconnected at junction 53. The areas of low fiber density 51 are disposed in first discontinuous portions 54 of the fabric with the discontinuous portions aligned in a square pattern so that they extend longitudinally and transversely of the fabric.

The discontinuous portions of the fabric are interconnected by ribbon-like groups 55 of fiber segments in second discontinuous portions of the fabric that define a plurality of areas of low fiber density 56 in third discontinuous fabric portions. The interconnecting groups contain highly aligned fiber segments. The interconnecting groups of fiber segments are disposed in the longitudinal and transverse directions of the fabric and at substantially the 12, 3, 6, and 9 o'clock positions at each of the second discontinuous portions 54 of the fabric.

The disposition of the interconnecting ribbon-like groups of fiber segments will depend upon two factors. One is the original fiber orientation in the starting fibrous web and the other is the pattern of the first discontinuous portions of the fabric. Generally, it can be said that the fiber segments in the interconnecting groups tend to align themselves in the direction of orientation of the starting fiber web. If an isoweb is used, the orientation in the starting web has little if any effect on how these fiber segments align themselves into the interconnecting groups. With regard to the pattern of the first discontinuous portions of the fabric, if these portions are aligned longitudinally and transversely of the fabric, the interconnecting groups in the second discontinuous portions of the fabric will be similarly aligned, while if these portions are staggered, the interconnecting groups will be disposed diagonally of the fabric.

Again, referring to FIG. 4 the areas of low fiber density of 51 in the first discontinuous portions 54 of the fabric have yet another pattern of yarn-like bundles 57 which extend across the areas of low fiber density of the first pattern. These yarn-like bundles 57 interconnect at substantially right angles with each other within the areas of low fiber density in the first pattern.

Referring to the diagrammatic showing in FIG. 5, the first discontinuous portions 60 of the fabric 61 are in a pattern of stripes which extend substantially across the entire width of the fabric. These stripes comprise areas of low fiber density 62 defined by yarn-like bundles 63 of fiber segments. The yarn-like bundles are con-

nected at junctures 64 by fibers common to a plurality of bundles. The stripes are connected to adjacent stripes of ribbon-like groups 65 of substantially aligned fiber segments. The groups 65 also extend across the entire width of the fabric.

#### DESCRIPTION OF MACHINE AND METHOD FOR MAKING FABRICS OF MY INVENTION

FIG. 6 shows one form of apparatus that may be used to produce the fabrics of the present invention. Full particulars of the basic apparatus of which this apparatus is a specific form, including methods of mounting, rotation, etc., are described in U.S. Pat. No. 2,862,251 issued Dec. 2, 1958, and are incorporated in the present application by reference and thus need not be described in complete detail here. In view of this reference, the apparatus of FIG. 6 will be described in general terms insofar as its essential elements are the same as in the patent just mentioned, and as already explained above, the features used to manufacture the novel non-woven fabrics of the present invention will be described in more detail.

The apparatus of FIG. 6 includes a rotatable perforated drum 70 suitably mounted on flanged guide wheels 71 and 72 which are mounted for rotation on shafts 73 and 74. The drum has apertures 75 uniformly spaced over its entire surface. Inside the drum, a stationary manifold 77 to which a fluid is supplied through conduit 78 extends along the full width of the drum. On one side of the manifold is a series of nozzles 79 for directing the fluid toward the drum.

A novel backing or supporting member 80 arranged to travel with rotatable drum 70 will be described below. (The term backing member and support member are used interchangeably throughout this description.)

Support member 80, as shown in FIG. 7, has a discontinuous pattern of formaminous portions 81 and a continuous pattern of imperforate portions 82 lying between and interconnecting them. In FIG. 7, the formaminous portions are round and arranged such that four of them lie in a square pattern over the surface of member 80. As already indicated above, the foraminous portions of the backing member may have any shape desired. They may also be arranged in any discontinuous pattern over the support member; i.e., they may be aligned longitudinally and/or transversely, staggered, etc.

FIG. 8 shows a cross-section of the backing means of FIG. 7 with a cross-section of apertured forming drum 70 included. As seen, each continuous imperforate portion 82 of backing means 80 has a curved top surface that rises slightly above the top surface of foraminous portions 81 of the backing means. Because of the curved top surface, central portion 85 rises above edge portions 86 of imperforate portion 82 of the backing means.

Rotatable drum 70 is solid throughout its area except for forming apertures 75 disposed across its surface. As already indicated above, these forming apertures may have any shape desired. They may also be arranged in any discontinuous pattern over the support member; i.e., they may be aligned longitudinally and/or transversely staggered, etc., with continuous land areas between them. In the apparatus of FIG. 6, forming apertures 75 are circular in shape and are arranged such that four of them lie in a square pattern over the surface of drum 70.

The diameter of circular apertures 75 is at least about ten times the average diameter of the fibers in the fibrous starting material. With fibers of 1½ denier, for example, the diameter of apertures 75 is 0.015" or larger.

Backing member 80 passes about drum 70 and separates from the drum at guide roll 90, which rotates on shaft 91. The belt passes downwardly around guide roll 92, rotating on shaft 93, and then rearwardly over vertically adjustable tensioning and tracking guide roll 94 rotating on shaft 95, and then around guide roll 96 on shaft 97. The member passes upwardly and around guide roll 98

rotating on shaft 99, to be returned about the periphery of the drum.

Drug 70 and backing belt 80 provide a rearranging zone between them through which a fibrous starting material may move to be rearranged, under the influence of applied fluid forces, into a non-woven fabric having a plurality of patterns of fiber segments that alternate and extend throughout its area.

Tension on backing belt 80 is controlled and adjusted by the tensioning and tracking guide roll. The guide rolls are positioned in slideable brackets which are adjustable to assist in the maintenance of the proper tension of the belt. The tension required will depend upon the weight of the fibrous web being treated and the amount of rearrangement and patterning desired in the final product.

Forming drum 70 rotates in the direction of the arrow shown, and backing belt 80 moves in the same direction at the same peripheral linear speed and within the indicated guide channels, so that both longitudinal and lateral translatory motion of the backing means, the apertured forming means, and the fibrous layer with respect to each other are avoided. The fibrous material 100 to be treated is fed between the drum and backing member 80 at point "A," passes through a fiber rearranging zone where fluid rearranging forces are applied to it, and is removed in its new, rearranged form as non-woven fabric 101 between the drum and belt at point "B."

As fibrous material 100 passes through the fiber rearranging zone, a liquid such as water is directed against the inner surface of forming drum 70 by nozzles 79 mounted inside the drum, the water passes through apertures 75 of forming means 70 into the layer of fibrous starting material 100 to produce rearrangement of the fibers of the web, and the water thence passes through foraminous portions 81 of backing means 80.

Vacuum assist box 102 is located against the outside surface of backing means 80. Vacuum box 102 has a slotted surface located closely adjacent the outer surface of belt 80, and through which suction is caused to act upon the web. Suction thus applied assists in the rearrangement of the fibers as the web material passes through the rearranging zone. In addition, it serves to help de-water the web and prevent flooding during fiber rearrangement. Vacuum box 103 located below drum 70 also helps de-water the web after it is rearranged.

In the apparatus of FIG. 6, the relative positioning of rotatable backing drum 70 and apertured forming means 80 with respect to the fibrous layer 100 being rearranged is maintained through the rearranging zone as explained above by guarding against either longitudinal or lateral translatory movement. This maintains the integrity of the rearranged fabric as it is subjected to fluid forces from the rearranging liquid.

The directions the streams of rearranging fluid projected through apertures 75 of drum 70 take as they move into and through the fibrous web determine the type of forces applied to the fibers and in turn, the extent of rearrangement of the fibers. Since the directions the streams of rearranging fluid take after they pass through apertures 75 are determined by foraminous portions 81 and imperforate portions 82 of backing means 80, it follows that the patterns of these portions of the backing means help determine the patterns of fiber arrangement, as well as the patterns of holes or other areas of low fiber density, in the resultant fabric.

With imperforate portions 82 raised only slightly above the foraminous portions of the backing means, it has been found that satisfactory formation of yarn-like bundles of fiber segments in the first pattern with areas of low fiber density delineated between the yarn-like bundles, can be achieved with a fibrous starting material made up of fibers of 1½ denier that has a web weight of no more than about 600 grains per square yard, or somewhat heavier for higher denier fibers. With a similar backing means and a fibrous starting material comprised of fibers of 1½ 75

denier of web weight of more than about 800 grains per square yard, it is ordinarily not possible to form such a pattern. The web weights in question may be somewhat higher for this kind of fiber rearrangement, the higher the 5 continuous imperforate portions rise above the discontinuous foraminous portions of the backing means.

FIG. 9 gives an enlarged fragmentary diagrammatic plan view of the foraminous portion 110 of another backing means that can be used with the apparatus of FIG. 6. 10 Foraminous portion 110 of the backing means for use in this invention is formed of coarse woven screen, preferably metal. In the embodiment shown, wires 111 running vertically in FIG. 9 are straight, while wires 112 running horizontally in that figure weave alternately over and 15 under wires 111. Protuberances 113 are present throughout foraminous portion 110 as the topmost part of each "knee" of a given strand 112 of the screen that is formed as the strand weaves over and under the strands 111 that lie perpendicular to it.

20 As a given strand 112 slants downward to pass under a strand 111 perpendicular to it, it crosses two other strands 112 disposed on either side of it, as those strands slant upward to pass over the same perpendicular strand that the given strand will pass under. Each series of such 25 "crossing points" 114 forms a trough, such as trough 115 formed by crossing points 114 in FIGS. 9 and 10, that lies between adjacent protuberances 113. The effective shape of troughs 115, as can be best seen in FIG. 10 (which shows a cross-section of element 110 of which a 30 plan view is given in FIG. 9), is substantially an inverted triangle.

35 A series of slightly deeper troughs 116 is formed between adjacent protuberances 113 but extending at right angles to troughs 115. As best seen in FIG. 11, the bottom of each trough 116 is formed by portions of straight strands 111, with successive protuberances 113 on each side of the trough forming the tops of the trough. As seen in FIG. 11, the effective shape of troughs 116 may 40 be characterized as a shallow U-shape.

45 As shown in FIG. 9, a plurality of troughs 115 and a plurality of protuberances 113 alternate in one direction across the surface of foraminous portion 110 of the backing means. FIG. 9 also shows that a plurality of troughs 116 and a plurality of protuberances 113 alternate in a direction perpendicular to troughs 115. Hence a plurality of troughs and a plurality of protuberances alternate in both the longitudinal and transverse directions across the 50 surface of foraminous portion 110 of the backing means.

55 Use in the apparatus of FIG. 6 of a backing means having foraminous portions such as element 110 shown in FIGS. 9 through 11 produces a third pattern of rearranged fibers within the areas of low fiber density of the first pattern corresponding to the apertures 75 in drum 70, such as is depicted in FIG. 4. This pattern within the first pattern is made up of yarn-like bundles of fiber segments that have been positioned in troughs 115 and troughs 116 on the surface of foraminous portion 110 of the 60 backing means.

65 If desired, a backing means such as element 110 may be used to produce the fabrics of the present invention by eliminating the apertured forming drum and projecting the rearranging fluid directly onto the fibrous web while it is supported on such a backing means. In such a method, the yarn-like bundles of fiber segments which define the areas of low fiber density in the first pattern have 70 been positioned in the troughs 115 and troughs 116 on the surface of the foraminous portions 110 of the backing means.

To produce satisfactory rearrangement of fibers into 75 yarn-like bundles of closely associated and substantially parallel fiber segments positioned in troughs 115 and in troughs 116, the vertical distance between the tops of protuberances 113 and the bottoms of the immediately adjacent troughs should be at least about three times, generally no more than about 15 to 20 times, and preferably

about five to about ten times, the average diameter of the fibers in the layer of fibrous starting material. For troughs 115, this distance is the vertical distance indicated in FIG. 10 by the pair of dashed lines that pass, respectively, through the tops of protuberances 113 and the crossing points 114 that define the troughs. The vertical distance from the bottom of each trough 116 to the tops of protuberances 113, on the other hand, is somewhat larger, being shown by FIGS. 10 and 11 to be equal to the diameter of a strand 112.

The relative position of a forming aperture 75 and protuberances 113 of foraminous portion 110 of the backing means in one form of the method and apparatus used to produce fabrics of this invention is shown in dashed lines in FIG. 9. As is seen, aperture 75, in both the longitudinal and transverse directions, has a width somewhat larger than two times the horizontal distance between the tops of immediately adjacent protuberances 113 on foraminous member 110 and spans two such protuberances measured in both the longitudinal and transverse directions.

The substantially aligned interconnecting fiber segments that form the second fiber pattern in the fabric of this invention are organized in flat, ribbon-like groups of fiber segments. These ribbon-like groups of fiber segments are formed by fiber segments which span each imperforate portion of the backing means and interconnect adjacent areas of the first fiber pattern. The location of such ribbon-like groups will depend for the most part on the pattern of discontinuous foraminous areas in the backing member and the fiber orientation in the starting material.

The rearranged web or fabric of this invention may be treated with an adhesive, dye or other impregnating, printing, or coating material in a conventional manner. For example, to strengthen the rearranged web, any suitable adhesive bonding materials or binders may be included in an aqueous or non-aqueous medium employed as the rearranging fluid. Or an adhesive binder may, if desired, be printed on the rearranged web to provide the necessary fabric strength. Thermoplastic binders may, if desired, be applied to the rearranged web in powder form before, during or after rearrangement, and then fused to bond the fibers.

The optimum binder content for a given fabric according to this invention depends upon a number of factors, including the nature of the binder material, the size and shape of the binder members and their arrangement in the fabric, the nature and length of the fibers, total fiber weight, and the like. In some instances, because of the strength of the fibers used or the tightness of their interentanglement in the rearranged web or fabric, no binder at all need be employed to provide a usable fabric.

Further details and description of methods and apparatus which may be used to produce the novel non-woven fabric of the present invention are given in my commonly assigned patent application entitled Method and Apparatus for Producing Non-Woven Fabrics Having a Plurality of Patterns (Case III) and Method and Apparatus for Producing Non-Woven Fabrics Having a Plurality of Patterns (Case V) filed concurrently with the present patent application. It is to be noted that not all embodiments of the apparatus disclosed in the above-mentioned patent applications will necessarily produce the novel non-woven fabric of the present invention.

The following are illustrative examples of the methods for producing the patterned nonwoven fabrics of the present invention:

#### Example 1

In apparatus as illustrated in FIG. 6, a web 100 of loosely assembled fibers, such as may be obtained by carding, is fed between apertured forming means 70 and backing means 80. The web weight is about 450 grains per square yard, and its fiber orientation ratio approximately 7 to 1 in the direction of travel. The web contains viscose rayon fibers approximately  $1\frac{1}{16}$ " long, of  $1\frac{1}{2}$  denier.

The apertured forming drum 70 used in this example has about 165 substantially round holes per square inch, each approximately 0.045" in diameter. The width of each of these apertures 75 is thus equal to about 30 times the 0.0015" average diameter of the  $1\frac{1}{2}$  denier fibers of the fibrous starting material. The holes are arranged in a diamond pattern over the forming drum. Each aperture 75 is spaced approximately 0.040" in the diagonal direction from the immediately adjacent aperture on the drum.

Backing means 80 in the apparatus used in this example is constructed of a woven nylon screen with a smooth surfaced flexible metal member having circular holes distributed across its surface in a diamond pattern adhered to the nylon screen.

This provides foraminous portions 81 in the backing means 80 which are comprised of a woven nylon screen of approximately 28 x 34 mesh, or substantially 952 openings per square inch. Each of these foraminous portions 81 has a diameter of approximately  $\frac{1}{4}$ ", with a space of approximately  $\frac{1}{8}$ " from each portion 81 to the nearest other portion 81 in a diagonal direction.

Discontinuous foraminous portions 81 are interconnected by the continuous metal portions. These continuous imperforate portions 82, in the area between each pair of immediately adjacent foraminous portions 81, have a central portion 85 that rises 0.012" above the plane of the top surface of discontinuous foraminous portions 81 of the backing means, and edge portions 86 that rise about 0.010" above the plane described.

Because of the indicated spacing of approximately  $\frac{1}{8}$ " between foraminous portion 81 of backing means 80, it follows that the width of each imperforate portion 82 at its narrowest part is about three times the width of an aperture 75 at its narrowest part.

Water is projected from nozzles 79 through apertures 75 in apertured forming means 70, and thence through fibrous web 100 and foraminous portions 81 of backing means 80.

After a given portion of fibrous web 100 passes through the rearranging zone, in which streams of water are directed against it as just described, the rotation (in the counterwise direction as seen in FIG. 6) of the sandwich comprised of apertured forming drum 70, the rearranged non-woven fabric 100, and backing member 80 brings the rearranged fabric to takeoff zone "B." There the rearranged non-woven fabric leaves the apparatus.

With the conditions indicated, good fiber rearrangement and bundling are obtained, and an excellent non-woven fabric such as shown in the photomicrograph of FIG. 1, which has a plurality of patterns that alternate and extend throughout the fabric, is produced.

Nonwoven fabric 20 of FIG. 1 contains a first plurality of areas of low fiber density 21 defined by yarn-like bundles 23 of fiber segments arranged in a first pattern corresponding to the discontinuous foraminous portions 81 of backing means 80. The nonwoven fabric also contains a second pattern of substantially aligned fiber segments 25 interconnecting the portions of the fabric in the first pattern 22. This second pattern corresponds to the configuration of continuous imperforate portions 82 of backing means 80.

The pattern of yarn-like bundles of fiber segments is arranged within the first portions 22 of the fabric in accordance with the pattern of land areas of apertured forming drum 70. Yarn-like bundles 23 define within these portions areas of low fiber density 21 arranged in accordance with the arrangement of apertures 75 in the apertured forming drum 70.

#### Example 2

FIG. 2 is a photomicrograph of another non-woven fabric made in accordance with the present invention by use of apparatus similar to that described in Example 1, but with a starting web of fibrous material of the type commonly called an isotropic web. The starting material has a web weight of about 350 grains per square yard,

## 13

and web strength is measured at substantially the same magnitude in every direction throughout the web. The web contains viscose rayon fiber approximately  $1\frac{1}{16}$ " long and 1½ denier.

The fabric of FIG. 2 is generally similar to the fabric of Example 1.

## Example 3

The starting material for this example is the same as in Example 2. Apertured forming drum 70 used in this example is the same as that in Example 1.

Backing means 80 in the apparatus of this example includes in part a smooth surfaced flexible plastic having foraminous circular portions distributed across its surface in a square pattern. Discontinuous foraminous portions 81 of backing drum 80 are comprised of a woven fiber glass screen of approximately 14 x 18 mesh or substantially 252 openings per square inch. Each of these foraminous portions has a diameter of approximately  $\frac{1}{4}$ ", with a space of approximately  $\frac{3}{32}$ " from each portion 81 to the nearest other portion 81 in a diagonal direction. Discontinuous foraminous portions 81 are interconnected by the continuous plastic portions of the backing belt.

Foraminous portions 81 of backing means 80 are formed as shown in FIG. 9 through 11. The vertical distance between the tops of protuberances 113 and troughs 115 such as shown in FIGS. 9 and 10 is approximately 0.005", or in other words a little more than three times the 0.0015" average diameter of the 1½ denier fibers making up the starting material for this example. The same vertical distance for troughs 116 such as those shown in FIG. 11 is slightly larger.

The horizontal distance between the tops of protuberances 113 is about 0.056" in one direction and about 0.071" in the other. These distances are equal, respectively, to about 37 times and about 47 times the 0.0015" average diameter of the fibers of the fibrous starting material. Each aperture 75 spans a plurality of protuberances 113 on the backing screen, measured in both the longitudinal and the transverse directions. Apertured forming drum 70 and backing belt 80 are spaced from each other during use of the apparatus of FIG. 6 to provide a fiber rearranging zone therebetween.

Use of the apparatus of this example produces a nonwoven fabric having a plurality of patterns of fiber segments that alternate and extend throughout the fabric. As seen in the schematic drawing of FIG. 4, nonwoven fabric 50 has a first pattern of yarn-like bundles of fiber segments 52 that define areas of low fiber density 51 all located within groups of fiber segments 54 arranged in accordance with the arrangement of discontinuous foraminous portions 81 of backing means 80. A second pattern of flat, ribbon-like groups of substantially aligned fiber segments 55 interconnects the portions of the fabric in the first pattern.

A third pattern of smaller yarn-like bundles of fiber segments 57 is positioned in troughs 115 and 116 of the foraminous portions of the backing means. These yarn-like bundles, lying within areas of low fiber density 51, subdivide those areas further into still smaller areas of low fiber density.

The above detailed description has been given for clearness of understanding only. No unnecessary limitations should be understood therefrom, as modifications will be obvious to those skilled in the art.

What is claimed is:

1. A nonwoven fabric with a plurality of patterns of groups of fiber segments that alternate and extend

## 14

throughout said fabric which comprises: a first pattern of yarn-like bundles of fiber segments defining a plurality of areas of low fiber density, said bundles being located in first discontinuous portions of the fabric, the fiber

5 segments in each of said bundles being closely associated with other fiber segments in the bundle and lying generally parallel to the longitudinal axis of the bundle, each of said yarn-like bundles of fiber segments being interconnected with other such bundles at junctures by groups 10 of fibers common to a plurality of bundles, the fibers at said junctures being oriented in a plurality of diverse directions, each pair of immediately adjacent first discontinuous portions of the fabric being interconnected by a ribbon-like group of substantially aligned fiber segments, said ribbon-like groups being located in second discontinuous portions of the fabric.

2. The nonwoven fabric of claim 1 in which each of said first discontinuous portions of the fabric extends continuously through the fabric in a given direction and 20 is parallel to and spaced from similar portions of the fabric, and in which each of said ribbon-like groups of substantially aligned interconnecting fiber segments also extend continuously through the fabric in said given direction.

25 3. The nonwoven fabric of claim 1 in which said ribbons of interconnecting fibers define a plurality of areas of low fiber density in third discontinuous portions of the fabric.

30 4. The nonwoven fabric of claim 3, in which the areas of low fiber density in said first discontinuous portions of the fabric are apertured substantially free of fibers.

5. The nonwoven fabric of claim 3 in which the areas of low fiber density in said third discontinuous portions of the fabric are apertures substantially free of fibers.

35 6. The nonwoven fabric of claim 3 in which other, smaller yarn-like bundles of fiber segments formed in the same manner as said first-mentioned yarn-like bundles of fiber segments extend across the areas of low fiber density in said first discontinuous portions of the fabric.

40 7. The nonwoven fabric of claim 6 in which said other, smaller yarn-like bundles of fiber segments are interconnected in the manner aforesaid with similar yarn-like bundles extending substantially at right angles thereto across the areas of low fiber density in said first discontinuous portions of the fabric.

## References Cited

| UNITED STATES PATENTS |           |         |                 |           |
|-----------------------|-----------|---------|-----------------|-----------|
| 50                    | 3,485,706 | 12/1969 | Evans           | 161—169 X |
|                       | 3,081,515 | 3/1963  | Griswold et al. | 28—78     |
|                       | 3,033,721 | 5/1962  | Kalwaites       | 161—150   |
|                       | 3,486,168 | 12/1969 | Evans et al.    | 161—169   |
| 55                    | 2,862,251 | 12/1958 | Kalwaites       | 19—161    |
|                       | 3,353,225 | 11/1967 | Dodson et al.   | 19—161    |
|                       | 3,403,862 | 10/1968 | Dworjanyn       | 239—566   |
|                       | 3,434,168 | 3/1969  | Summers         | 28—72.2   |
|                       | 3,485,708 | 12/1969 | Ballou et al.   | 161—72    |
| 60                    | 3,494,821 | 2/1970  | Evans           | 161—169   |
|                       | 3,498,874 | 3/1970  | Evans et al.    | 161—169 X |

ROBERT F. BURNETT, Primary Examiner

R. L. MAY, Assistant Examiner

65 U.S. CL. X.R.

19—161 P; 28—72.2; 161—169